

# UNITED STATES PATENT OFFICE.

ROGER WILLIAMS, OF PROVIDENCE, RHODE ISLAND, ASSIGNOR TO NITROGEN PRODUCTS COMPANY, OF PROVIDENCE, RHODE ISLAND, A CORPORATION OF RHODE ISLAND.

## PROCESS OF AND MEANS FOR FIXING ATMOSPHERIC NITROGEN.

1,314,231.

Specification of Letters Patent. Patented Aug. 26, 1919.

No Drawing.

Application filed October 28, 1917. Serial No. 198,711.

To all whom it may concern:

Be it known that I, ROGER WILLIAMS, a citizen of the United States, residing at Providence, in the county of Providence and 5 State of Rhode Island, have invented certain new and useful Improvements in Processes of and Means for Fixing Atmospheric Nitrogen, of which the following is a specification.

10 This invention relates to a process of and means for fixing atmospheric nitrogen and more especially to an improvement in or upon the process disclosed in the patent to John E. Bucher, No. 1,120,682, dated Dec. 15 15, 1914; the present invention having for one of its objects the effectuation of said Bucher process in such manner as to increase the efficacy thereof, both as regards the conversion of carbonate of sodium, or the like, 20 to cyanid, and also as regards the mechanical feeding of the preferably briquetted charge through the cyanizing retort.

Another object of my invention is to produce a composition of matter in briquetted 25 form, which shall be more resistant to disruption and fracture, when cold, and more resistant to deformation and disintegration of its briquetted structure when under operative temperature and pressure conditions to 30 which it must be subjected when in use; while at the same time in substantially no way impairing the efficiency of the briquets for the formation of cyanid therein,—but, on the contrary, actually improving them 35 for this latter purpose.

These and other objects will be herein-after referred to, and the novel combinations of steps in the process and of elements in the briquet structure, will be more particularly pointed out in the claims appended 40 hereto.

As I am aware of certain modifications and changes which may be effected herein, without departing from the spirit of my invention, I desire to be limited only by the 45 scope of said claims, broadly interpreted in the light of my disclosure.

As described in detail in said Bucher patent, the preferred mode of effectuation of his said process is by preparing relatively 50 small briquets of reactive material, which includes iron, finely divided—or some equivalent catalytic material, *e. g.* chrom-

ium, manganese, nickel or cobalt,—very intimately mixed with carbon and a substance such as sodium carbonate which acts not alone as a binder for the briquets; but also as a source of the metal which constitutes the base of the cyanid or other cyanogen compound to be formed. These briquets may be fed into a suitable retort and after being preheated, descend by gravity, or are otherwise moved into a heat zone where free nitrogen is caused to react upon the briquetted material to convert a considerable portion of the carbon and sodium carbonate or its equivalent, to sodium cyanid. In this reaction, the iron, or the like, acts catalytically and the operation is conducted at a temperature which preferably never is allowed to exceed the eutectic point of said catalyst. In practice the operating temperature is approximately 1000° C. or somewhat higher, when iron is the catalyst employed; but aside from the likelihood of 75 injuring the catalyst,—since the sodium carbonate or its equivalent, constitutes the binder for the briquets, it is highly undesirable to so elevate the temperature of the entire reactive mass, at any one time, as to excessively volatilize this binder. This, of course, is due to the fact that the briquet structure must be reasonably preserved in order to afford the requisite passages or ducts for the passage of the nitrogen through the mass and the elimination from the pores of said mass of the carbon monoxid formed during the course of the reaction; and also to prevent the charge from sticking in the retort. 90

With briquets formed as described in said patent to Bucher, however, I have discovered that there is a tendency for them to become over-plastic and, indeed at times in consequence thereof to thus cut off more or less of the requisite nitrogen supply and even to choke the retorts, especially when operating at a temperature well up above 1000° C. (*e. g.* 1090° C.); the binder then being excessively liquefied and thereafter volatilized. If now this liquid were converted to a rather thick paste, so to speak, by the presence therein of an exceedingly finely divided and preferably highly porous, irregularly surfaced material, this excessive fluidity and volatilization of melted portions 100

of the sodium carbonate binder would be in part overcome. The difficulty was, however, to find such a substance, which would not be instrumental in introducing into the 5 reactive mass impurities which the novel employment by said Bucher, of the sodium carbonate itself as the preferably sole binder for the briquets, avoided.

Peculiarly, such a substance as most 10 admirably meets the requirements, is actually evolved during the course of the operation as described in said patent; but was used merely to augment the supply of carbon in the briquets after they had already been 15 formed and had been introduced into the furnace. I refer to the carbon deposited in the pores of and upon the briquets, from the conversion of the carbon-monoxid produced by the reaction (supplemented by additional CO, if desired, in the manner described in said Bucher patent) into carbon-dioxide in a zone or region in the retort or hopper, where the temperature of said carbon-monoxid was lowered sufficiently to permit 20 of the conversion of much of said monoxid to the dioxid.

This carbon, as is stated in said patent, is ash-free and is for this and other reasons 30 particularly well suited to the cyanid forming operation; the briquets upon which it is deposited or in the pores of which it is formed, dropping by gravity into the heat zone, where after being cyanized, they are cooled and preferably then removed from 35 the retort, to be treated to win the cyanid therefrom.

This operation, as formerly conducted, involved the lixiviation of the cyanized 40 briquets with water, which dissolved out the cyanid and also, unfortunately, the sodium carbonate as well. The briquets hence became converted to a black sludge from which the iron segregated, while, of course the greater part of the carbonate was removed 45 therefrom in solution, to be recovered by subsequent treatment. The sludge which was largely carbon, was dried and of course caked into masses and lumps which were subsequently ground up and again mixed 50 with iron and sodium carbonate, preparatory to being re-briqueted.

Now it so happens that the carbon which is deposited in the pores of the briquets by the conversion of CO to CO<sub>2</sub>, as above described, is usually by no means wholly consumed in the subsequent cyanid forming operation; but by the just described lixiviation and other treatment of the briquets, this material is practically lost to the process in 55 so far as its peculiarly finely divided and hence reactive condition is concerned.

When, however,—instead of lixiviating the cyanized briquets with water,—they are extracted with liquid ammonia, this substance 60 dissolves with ease the alkali metal

cyanid and exerts practically no solvent action upon the alkali metal carbonate or hydrate, especially if no water be present in either the briquets being treated or in the leaching agent. I may here observe that 70 since even a small percentage of water in the liquid ammonia solvent exercises a marked influence upon the solubility of, for example, sodium hydrate therein, I greatly prefer to carefully exclude, as far as possible, all traces of moisture during this extracting operation.

As, by the use of this solvent, the briquets are no longer converted to sludge,—the exceedingly finely divided condition of the 80 precipitated carbon is not impaired and it is merely necessary to conserve it, preferably as far as practicable, during the removal of the leached and thoroughly dry briquets from the leaching or extracting apparatus, 85 and thereafter during the subsequent breaking up of the briquets preparatory to adding fresh carbonate and carbon to the material prior to the re-briquetting operation.

I may also observe that by operating in 90 this fashion, the segregation of the pulverulent catalyst, *e. g.* iron or its equivalent, is avoided; which materially reduces the time and cost of preparing the intimate mixture of carbon, catalyst and carbonate or the 95 like, required for the cyanizing step or operation.

If care be not observed, however, and the leaching or extracting apparatus is opened and the charge is dropped therefrom, especially when out of doors or in a building 100 the doors and windows of which are open for any reason,—then much of this very fine carbon dust will be blown away or float off in the air and be completely lost to the 105 process.

I hence prefer to conduct all such steps in a fashion to conserve this valuable substance; hoods or the like being used in a known manner to collect the carbon dust to 110 the end that it may be returned to the process.

Not alone is its presence in the briquets, mixed with iron or the like and coarser carbon particles, *i. e.* pulverulent coke,—of 115 value in aiding the alkali metal carbonate, or its equivalent, to bind the briquetted materials firmly together; but it is truly ash-less and free from silicates, sulfur and other deleterious impurities, which more or 120 less contaminate the product (cyanid). Could the entire supply of carbon in the briquets conveniently or practicably be made solely of this ash-free carbon, the condition would be ideal. However, it has not 125 yet been proven commercially practicable so to do; although I am at present at work upon this problem. On the other hand coke obtained from coal, such as has hitherto been used in the process, is always impure 130

and its content of ash runs from three or four per cent. (from specially selected anthracite coke) up to seven or eight per cent. or more.

5 Other sources of available carbon tried, were correspondingly subject to this objection, which has proven rather a serious one, not because the presence of ash materially interferes with the cyanizing operation; but 10 because it makes the final product impure. I have, however, also succeeded in practically overcoming this difficulty, by the use of what is known as petroleum coke,—a product obtained by coking down heavy 15 mineral oils,—and when this coke is finely pulverized, it more nearly resembles gaseous-reaction precipitated carbon such as that above described, than any other of which I am aware, which is commercially practicable. Its content of ash, if of reasonably 20 good quality, ranges from less than one-quarter of one per cent. to at times one and one-half per cent.; the average being perhaps, one per cent. The crushed particles 25 thereof, further, seem to be finer and more adapted to the purpose in question than those of similarly treated ordinary coke or the like.

30 Hence, when carbon is added to the briquet material, I prefer to use the combination of finely pulverized petroleum coke, and as much of the precipitated carbon, or its equivalent, as is available. The briquets are preferably prepared from a very intimate 35 mixture of, say, equal parts of catalyst, carbon and reactive binder; the catalyst being pulverized manganese, iron, or other equivalent catalytic material; the carbon comprising finely crushed, high-grade, petroleum coke and all available precipitated 40 carbon, produced as aforesaid; and the binder being preferably an alkali metal compound such as the carbonate, hydrate or 45 oxid of sodium, or a mixture of these, in which mixture the carbonate preferably principally predominates.

The said intimate mixture is then slightly moistened; care being taken to add but substantially just sufficient water (either as liquid or in the form of steam) to enable the binding material to become effective as such, and not to unduly mush-up or cake the exceedingly fine carbon particles. If, 50 too, more water is added than is necessary, then some of the catalyst, especially if iron is used as the catalytic material,—is apt to become partly oxidized, and while the subsequent cyanid forming operation will 55 quickly reduce this oxid to metal; still, heat and carbon are consumed in so doing and the effectiveness of the catalyst, until reduced, is impaired.

The mass is then briqueted by pressure in 60 suitable apparatus, and after it has been

slowly and thoroughly dried, it is available for use in the retort.

Obviously, also, the carbonate or the like may be fused to cause it to become effective as a binder when the material is briqueted; 70 instead of forming the briquets by means of water, as above described. The first method is preferred, however, and, when but little water is thus used, this can be very readily driven off in the drying operation. 75

I do not as yet know, with certainty, just why the presence of the precipitated carbon and crushed petroleum coke in the binder increases the rigidity and resistance to crushing or rupture of the briquets, when 80 cold,—as compared to briquets prepared in the same manner but with ground coke (from coal) instead of the preferred carbonaceous material; and it may be that my theory, aforesaid, regarding the action of 85 the precipitated carbon in connection with the partly molten binder, when the briquets are being cyanized, is incorrect. Be that as it may, however, the briquets prepared in accordance with my disclosure herein, are better able to resist fracture when cool or comparatively cool, and deformation or mashing up when in the heat zone; while they feed through the retort much more readily,—the 90 tendency to stick in or choke the retort being markedly reduced. I may here state also, that the briquets are handled, mechanically or otherwise, even more when cold than when hot. 95

The efficiency of this important nitrogen fixation process is therefore considerably enhanced by the herein described improvement; and as I am aware that other carbonaceous material in an extremely finely 100 divided and rough or porous surfaced condition is available for use in the process, I do not desire to be limited solely to crushed petroleum coke and the carbon precipitated during the conversion of carbon monoxid to 105 carbon dioxid; although these materials are 110 much preferred.

To this end, in certain of the appended claims such expressions as "substantially pure carbon as produced in and deposited 115 from gaseous material", are intended to cover the preferred carbon precipitated from carbon monoxid, as aforesaid, and also the carbon deposited in the flues which carry off the combustion products resulting from 120 the production of sodium carbonate, and the like; carbon obtained from the dissociation of partial decomposition of methane or other hydro-carbons; etc.

In general, carbon so produced or liberated by chemical reaction in gaseous materials, and when not excessively contaminated by impurities, is particularly available for use in the process on account not alone of its ultra-finely divided condition; but, fur- 125 130

ther, on account of the rough or irregular and peculiarly porous surfaces of its particles. On the other hand, ordinary coke, obtained from coal, normally has not only a high ash content, but further is so resistant to fracture,—especially when the fragments have been reduced to small size,—that when subjected to crushing and pulverizing action, they tend to shape themselves into minute ball-like masses the surfaces of which are relatively smooth and comparatively non-porous; certainly as compared to carbon precipitated from gaseous reaction residues.

15 I am of the opinion also, that there is another relationship between this irregularly surfaced ultra-finely divided carbon and the treatment with water, of the mixture to be briquetted; in that if it be subjected to too much water, the exceedingly minute pores in the surfaces of the carbon particles tend to become choked up. When, however, but just sufficient water is employed, as above described, it is probable that when this is evaporated off after briquetting, the carbon particles, while being knit or bound securely together, nevertheless have more or less open pores in their surfaces and,—as they are substantially in contact with each other,—the given briquet comprising them, is provided with a relatively complete system of tiny ducts or conduits for the passage of nitrogen therethrough and the emergence of the cyanid-reaction-retarding carbon monoxid therefrom.

For a number of reasons, therefore, the importance of eliminating water as a means for removing the cyanid from cyanized briquets,—where the solid residues are to be again incorporated in briquets, for return to the process,—will be appreciated. I make no claim herein, however, to liquid ammonia, *per se*, as a leaching agent, other than as this solvent co-acts with my preferred source of carbon for the cyanid forming operation, to enable the preservation and conservation of such carbon, in the manner described.

Finally, I desire to point out that while in the preferred mode of effectuating the process I prefer to use an alkali metal compound, such, for example, as sodium carbonate, as the source of the base of the cyanogen compound to be formed,—in certain of its aspects, my invention is not to be regarded as being limited to these, as I am aware that the nitrogen-fixing reaction may be effectuated by the use of, for example, compounds of the earth-alkali metals, such as barium carbonate; and further that the mixture of reactive material (carbon, catalyst and carbonate or the like) may have as its entire content of carbon, if desired, such ultra-finely divided material as the precipitated carbon, aforesaid.

I have this in view because of a process which I have developed for producing this substance outside of the briquet mass disposed in the relatively cool zone above the heat or cyanid-forming reaction zone in the nitrogen fixing operation,—and I anticipate being able to render said process, thus in view, not merely practicable on a small scale but in a commercially practicable way.

There are, however, certain advantages to be gained from using a mixture of such carbon with, preferably, petroleum coke powder; the latter for one thing, usually having in the particles thereof relatively larger pores than those of the precipitated carbon; while, as aforesaid, the finer carbon tends, when present in sufficient quantity, to form a paste, so to speak, with the binder-compound, and hence the advantage of extreme porosity is combined with greater resistance to rupture or deformation, as aforesaid.

Having thus described my invention, what I claim is:

1. In a process for fixing nitrogen in the form of a metal cyanogen compound, in which free nitrogen is caused to react upon briquets comprising catalytic material in finely divided condition, carbon and a substance which constitutes both the source of the metallic base of said cyanogen compound and a binder for said briquets,—the improvement which consists in incorporating directly into the binder of and during the operation of forming said briquets, as a source of carbon for the nitrogen-fixing reaction, carbonaceous material which comprises substantially pure flocculent carbon as produced in and deposited from gaseous material.

2. In a process for fixing nitrogen in the form of a metal cyanogen compound, in which free nitrogen is caused to react upon briquets comprising catalytic material in finely divided condition, carbon and a substance which constitutes both the source of the metallic base of said cyanogen compound and a binder for said briquets,—the improvement which consists in incorporating directly into the binder of and during the operation of forming said briquets, as a source of carbon for the nitrogen-fixing reaction, carbonaceous material which comprises carbon particles, in an ultra-finely divided state, obtained from the conversion of carbon monoxid to carbon dioxid.

3. In a process for fixing nitrogen in the form of a metal cyanogen compound, in which free nitrogen is caused to react upon briquets comprising catalytic material in finely divided condition, carbon and a substance which constitutes both the source of the metallic base of said cyanogen compound and a binder for said briquets,—the improvement which consists in incorporating directly into the binder of and during

- the operation of forming said briquets, as a source of carbon for the nitrogen-fixing reaction, carbonaceous material which comprises carbon particles, in an ultra-finely divided state obtained from a gaseous reaction in which said carbon particles are thrown out of and tend to separate from the gaseous reaction residues, so removing said cyanogen compound from said briquets, after its formation as aforesaid, as to leave such of said carbonaceous material as remains unchanged by the cyanid-forming reaction, in substantially said ultra-finely divided state, conserving such residual carbonaceous material and returning it to the process incorporated in fresh briquets.
4. In a process for fixing nitrogen in the form of a metal cyanogen compound, in which free nitrogen is caused to react upon briquets comprising catalytic material in finely divided condition, carbon and a substance which constitutes both the source of the metallic base of said cyanogen compound and a binder for said briquets,—the improvement which consists in incorporating directly into the binder of and during the operation of forming said briquets, as a source of carbon for the nitrogen-fixing reaction, carbonaceous material which comprises carbon particles, in an ultra-finely divided state, obtained from a gaseous reaction in which said carbon particles are thrown out of and tend to separate from the gaseous reaction residues, removing said cyanogen compound from said briquets, after its formation as aforesaid, by leaching said briquets with liquid ammonia, so as to leave such of said carbonaceous material as remains unchanged by the cyanid forming reaction, in substantially said ultra-finely divided state, conserving such residual carbonaceous material and returning it to the process incorporated in fresh briquets.
5. In the manufacture of briquets for use in the process which involves reacting with free nitrogen upon material in the form of briquets which comprise catalytic metal in finely divided condition, carbon and a reactive binding material,—the improvement which consists in mixing with said catalytic metal and binding material, petroleum coke in finely divided condition and substantially ash-free carbon obtained by converting carbon monoxid to carbon dioxid, treating the resulting mixture with substantially the minimum quantity of water necessary to enable it to be effectually briquetted, forming it into briquets, and driving off the water by heat.
6. In the manufacture of briquets for use in the process which involves reacting with free nitrogen upon material in the form of briquets which comprise catalytic metal in finely divided condition, carbon and a reactive binding material,—the improvement

which consists in mixing with said catalytic metal and binding material, substantially ash-free carbon obtained by converting carbon monoxid to carbon dioxid, treating the resulting mixture with substantially the minimum quantity of water necessary to enable it to be effectually briquetted, forming it into briquets, and driving off the water by heat.

7. In the manufacture of briquets for use in the process which involves reacting with free nitrogen upon material in the form of briquets which comprise catalytic metal in finely divided condition, carbon and a reactive binding material,—the improvement which consists in mixing with said catalytic metal and binding material, substantially pure carbon as produced in and deposited from gaseous material, treating the resulting mixture with substantially the minimum quantity of water necessary to enable it to be effectually briquetted, forming it into briquets, and driving off the water by heat.

8. The process of fixing nitrogen which comprises reacting with free nitrogen upon a briquetted mixture of catalytic metal, substantially ash-free carbon and the carbonate of an alkali metal, to form an alkali metal cyanogen compound, cooling the non-gaseous products of said reaction while preventing access of moisture thereto, extracting said cyanogen compound by liquid ammonia from which substantially all moisture is excluded, conserving the residue of said carbon and incorporating the same in fresh briquets for return to the process.

9. The process of fixing nitrogen which comprises reacting with free nitrogen upon an intimate mixture of catalytic material, finely crushed petroleum coke and an oxygen compound of an alkali metal capable of reacting with the substances aforesaid to form the cyanid of said alkali metal, cooling the non-gaseous products of said reaction while preventing access of moisture thereto, extracting said cyanogen compound by liquid ammonia from which substantially all moisture is excluded, and conserving the residue of said carbon for return to the process.

10. The process of fixing nitrogen which comprises reacting with free nitrogen upon an intimate mixture of catalytic material, finely crushed petroleum coke and an oxygen compound of an alkali metal capable of reacting with the substances aforesaid to form the cyanid of said alkali metal, cooling the non-gaseous products of said reaction while preventing access of moisture thereto, and extracting said cyanogen compound by liquid ammonia from which substantially all moisture is excluded.

11. The process of fixing nitrogen which comprises reacting with free nitrogen upon an intimate mixture of catalytic material, finely crushed petroleum coke and an oxygen

compound of an alkali metal capable of reacting with the substances aforesaid to form the cyanid of said alkali metal.

12. The step in an improved process for fixing nitrogen, which comprises forming a mixture of petroleum coke, sodium carbonate and catalytic material capable, when said mixture is heated to reacting temperature in the presence of free nitrogen, of combining said nitrogen with carbon from said petroleum coke and with the metal of said carbonate.

13. An improved briquet for nitrogen fixation purposes, which comprises petroleum coke, finely divided iron and sodium carbonate, the pores of said petroleum coke being substantially open and relatively free from said carbonate.

14. An improved briquet for nitrogen fixation purposes, which comprises finely divided petroleum coke, mixed with still more finely divided carbon obtained from the conversion of carbon monoxid to carbon dioxid, finely divided iron and sodium carbonate, the latter acting as the binder for said briquet.

15. An improved briquet for nitrogen fixation purposes, which comprises substantially pure flocculent carbon as produced in and deposited from gaseous material, finely divided catalytic material and a binder-forming compound which acts both as a binder for said briquet and as a source of the metal which constitutes the base of the nitrogen compound to be formed, said carbon being present in such quantity in and so intimately commingled with said binder-forming compound that, when the latter is liquefied by heat, said carbon forms a paste therewith.

16. An improved briquet for nitrogen fixation purposes, which comprises flocculent carbon, finely divided iron and sodium carbonate, the pores of said carbon being substantially open and relatively free from said carbonate.

In testimony whereof I have affixed my signature, in the presence of two witnesses.

Witnesses:

HOWARD F. HYLAND,  
HOWARD C. RIPLEY.

ROGER WILLIAMS.